



US006544709B1

(12) **United States Patent**  
Wang et al.

(10) **Patent No.:** **US 6,544,709 B1**  
(45) **Date of Patent:** **Apr. 8, 2003**

(54) **GLOSSY ELECTROPHOTOGRAPHIC MEDIA  
COMPRISING AN OPAQUE COATED  
SUBSTRATE**

(75) Inventors: **John Wang**, Lincoln, RI (US); **George Wu**, W. Warwick, RI (US); **Janice Lee Chin**, Westborough, MA (US)

(73) Assignee: **Arkwright, Inc.**, Fiskeville, RI (US)

(\*) Notice: Subject to any disclaimer, the term of this patent is extended or adjusted under 35 U.S.C. 154(b) by 0 days.

(21) Appl. No.: **10/036,785**

(22) Filed: **Oct. 19, 2001**

(51) **Int. Cl.<sup>7</sup>** **G03G 13/20**; B32B 9/00

(52) **U.S. Cl.** **430/124**; 428/195; 428/413; 428/480; 428/484

(58) **Field of Search** **430/124; 428/195, 428/413, 480, 484**

(56) **References Cited**

U.S. PATENT DOCUMENTS

5,055,371 A 10/1991 Lee et al. .... 430/126  
5,104,721 A 4/1992 Sun ..... 428/206  
5,145,749 A 9/1992 Matthew ..... 428/511

5,208,093 A 5/1993 Carls et al. .... 428/195  
5,208,211 A 5/1993 Kurotori et al. .... 503/227  
5,837,351 A 11/1998 Chernovitz et al. .... 428/195  
5,846,637 A 12/1998 Malhotra et al. .... 428/195  
5,989,686 A 11/1999 Song et al. .... 428/195  
6,177,222 B1 1/2001 McAneney et al. .... 430/124

FOREIGN PATENT DOCUMENTS

EP 0 633 508 B1 9/2001

OTHER PUBLICATIONS

US 5,032,440, 7/1991, Takeuchi et al. (withdrawn)

*Primary Examiner*—Mark A. Chapman

(74) *Attorney, Agent, or Firm*—Barlow, Josephs & Holmes, Ltd.

(57) **ABSTRACT**

The invention relates to electrophotographic recording media suitable for use with color copiers and laser printers. The media comprise an opaque substrate coated with a toner-receptive layer containing an epoxy or polyester resin having a melting point in the range of about 105° C. to about 200° C., and a wax having a melting point in the range of about 90° C. to about 200° C. The glossy media have good blocking resistance and are capable of producing high quality colored images.

**20 Claims, No Drawings**

**GLOSSY ELECTROPHOTOGRAPHIC MEDIA  
COMPRISING AN OPAQUE COATED  
SUBSTRATE**

**BACKGROUND OF THE INVENTION**

**1. Field of the Invention**

The present invention relates to electrophotographic recording media suitable for use with toner printing systems such as copiers and laser printers. Particularly, the media comprise an opaque substrate material coated with a toner-receptive layer.

**2. Brief Description of the Related Art**

In recent years, consumers and businesses have turned to electrophotographic printing systems (e.g., color copiers and color laser printers) to produce digital photographic images on a variety of products. Consumers and businesses can now create digital color images on greeting cards, posters, calendars, newsletters, business cards, advertising brochures, and the like. Manufacturers have introduced new digital cameras, computers, software, color copiers, color laser printers, and imaging media to meet growing demand in the home and business markets.

Generally, in an electrophotographic printing process, toner is used to form an image (i.e., photo, illustration, text, and the like) on a recording medium. Typically, the recording medium comprises a specially coated paper or film substrate. The toner comprises a binder resin and colorant particles, and it is magenta, cyan, yellow, or black colored. The process involves electrically charging a photoconductive surface of a drum or belt in the printing device (copier, printer, etc.). Light is directed at the photoconductive surface to form a latent image. The latent image on the photoconductive surface comprises electrostatic charges replicating the image that will be printed onto the medium. Toner particles are brought into contact with the photoconductor, and the particles are attracted to the charged regions on the photoconductive surface. As the recording medium passes over the toner-containing photoconductive surface, the toner particles are transferred to the medium. The toner image then can be fixed by briefly heating the medium. The heat fuses the toner to the medium creating a final imaged product.

Typically, in the fusing step, the medium passes between heated fuser rollers. Many color copiers and color laser printers contain fuser rollers coated with oil (e.g., silicone oil) to prevent smearing of the image and sticking of the imaged medium to the surface of the roller. For example, the Xerox Docucolor 12 color copier contains such oil-coated fuser rollers. However, such oil-based copiers and printers can have high maintenance costs. Recently, copiers and printers that do not use oil in their fusing stations have been introduced. Several popular models of color laser printers, such as Hewlett Packard (HP) 4500 and Xerox Phaser 790, do not contain oil-coated fuser rollers.

The quality of the printed image is dependent on many factors including the composition of the paper or film media. There is a growing demand for media that can produce digital images of similar quality to traditional photographic camera prints. For example, traditional photo developing machines create a glossy finish on the photo print. Many consumers find the glossy finish of conventional photo prints appealing. High gloss digital photo prints would also be desirable.

McAneney et al., U.S. Pat. No. 6,177,222 B1 discloses photographic papers suitable for use in electrophotographic

imaging systems. The paper is coated with a polyester coating having a thickness of about 1 to about 15 microns. According to the patent, the polyester coating absorbs the fused toner particles, thereby resulting in a smooth imaged surface. The patent describes the paper as capable of forming a glossy image, wherein the gloss is uniform across the image. Particularly, the images have a gloss value from about 50 GU to about 100 GU and a gloss variation between about 20 GU to about 10 GU.

10 Cobum et al., U.S. Pat. No. 6,060,203 discloses coated papers for producing photographic-like output having a uniform glossy finish in an electrostatographic printing process. The printing system comprises: a) a toner comprising a polyester resin having a glass transition temperature (T<sub>gt</sub>), and b) a coated substrate comprising a polyurethane, acrylic, or styrene-acrylic copolymer-based coating having a glass transition temperature (T<sub>gc</sub>). The patent discloses that good results are obtained when (T<sub>gc</sub>) is less than or equal to (T<sub>gt</sub>). The patent further discloses that coatings having high gloss values of 60 to 95% after fusing are preferred.

15 Chernovitz et al., U.S. Pat. No. 5,837,351 discloses a multi-purpose sheet suitable for use in manual drafting, ink-jet and electrophotographic printing and copying applications. The sheet comprises a base support coated with an aqueous dispersion of a cross-linkable polymer, a cross-linking agent, and pigment. The patent describes transparent vellum paper, film, and opaque paper as suitable base supports. The patent describes bisphenol A-based epoxy resins as suitable cross-linkable polymers and silica, silicate, and calcium carbonate as suitable pigments. According to the patent, the cross-linkable binder polymers coalesce and cross-link to produce a hard discrete surface layer that is ink-wettable and has controlled surface resistivity.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9

Cellulosic materials or polymeric films are suitable opaque substrates. The epoxy resin can be derived from bisphenol A and epichlorohydrin, and the wax can be hydrocarbon (e.g., polyethylene or polypropylene), hydrohalocarbon, ester-containing, synthetic, or natural (e.g., carnauba) waxes. Suitable anti-static agents include cationically and anionically conductive polymers. The toner-receptive layer can further comprise pigment particles such as silica, calcium carbonate, kaolin, aluminum hydroxide, starch, polystyrene, and poly(methyl methacrylate) particles. The coat weight of the toner-receptive layer can be in the range of about 1 to about 15 grams per square meter (gsm). The substrate can have a thickness in the range of about 50 microns (2 mils) to about 200 microns (8 mils).

In one embodiment, the back surface of the medium is also coated with the above-described toner-receptive layer so that the medium is capable of being imaged on either of its surfaces.

The present invention also encompasses a process for producing an image on the electrophotographic recording medium. The process comprises the steps of: a) providing an electrophotographic recording medium as described above; b) applying toner to form an image on the surface of the medium; and c) treating the medium with heat to fuse the toner to the medium. The recording medium can be passed between oil-coated or non-oil-coated heated rollers to fuse the toner to the medium.

#### DETAILED DESCRIPTION OF THE INVENTION

The present invention relates to an electrophotographic recording medium comprising an opaque substrate having a front surface coated with a toner-receptive layer. The layer comprises a resin selected from the group consisting of epoxy and polyester resins having a melting point in the range of about 105° C. to about 200° C., and wax having a melting point in the range of about 90° C. to about 200° C. The amount of wax in the layer is no greater than 14% by weight based on total weight of the layer. The recording medium has a surface gloss of at least 70 GU as measured by a 60 degree glossmeter.

Any suitable substrate material can be used provided that the material is substantially opaque. By the term, "opaque", as used herein, it is meant that the opacity of the material is at least 70%. Opacity can be measured with a BNL Opacimeter (available from Technidyne Corp., New Albany, Ind.) using standard procedures described in the instrument manual provided by the manufacturer.

For example, opaque polymeric films comprising a polymer such as polyester, polymethylmethacrylate, polyethylene, polystyrene, polyvinylidene fluoride, polyvinyl chloride, polyamide, and polyimide can be used. Alternatively, opaque cellulosic substrates are suitable. For example, papers made from blends of hardwood and softwood fibers are suitable. The papers can contain various sizing agents, pigments, and fillers and be latex-impregnated. Suitable paper substrates are commercially available under various tradenames from companies such as Consolidated Papers, Mohawk Paper Mills Inc., P.H. Glatfelter Company and Garda Cartiere. The manufacturer of the opaque cellulosic substrate may coat the surface of the substrate with polymers such as polyethylene or polypropylene to provide a moisture barrier layer on the surface of the substrate. The coating may enhance surface glossiness of the substrate. The coatings can be formed by extruding the

coating composition onto both surfaces (front and back) of the cellulosic substrate. Such "poly-coated" papers are commercially available from companies such as Jen-Coat, Inc. and Felix Schoeller Technical Papers, Inc. Other opaque substrate materials, such as TYVEK (spun-bonded polyolefin) which is available from the DuPont Company, may be suitable.

The thickness of the opaque substrate is not particularly restricted but should generally be in the range of about 50 microns (2 mils) to about 200 microns (8 mils). The opaque substrate has two surfaces. The first surface, which is coated with a toner-receptive layer, may be referred to as the "front surface" or "imaging surface", and the opposite surface may be referred to as the "back surface".

The toner-receptive layer comprises an epoxy or polyester resin having a melting point in the range of about 105° C. to about 200° C. and preferably in the range of 110° C. to 170° C. Suitable epoxy resins include EPON 1007F and EPON 1009F available from Shell Chemical Company. These

epoxy resins are derived from bisphenol A and epichlorohydrin. Preferably, the toner-receptive layer comprises an epoxy or polyester resin in an amount of at least about 80% by weight based on total dry weight of the toner-receptive layer. The melting point of the resin may be provided in technical data sheets available from the manufacturer. Melting points can be determined by techniques known in the art such as differential scanning calorimetry, a ring and ball softening test, or testing methods such as ASTM D-3461 as noted in the below Examples.

Further, the toner-receptive layer contains a wax having a melting point in the range of about 90° C. to about 200° C. Preferably, the melting point is in the range of about 90° to about 150° C. Waxes can have a partially crystalline structure and melt over a relatively narrow temperature range. But, some waxes have a more amorphous structure and will melt over a relatively broad range. The melting point of the wax may be provided in technical data sheets available from the manufacturer. Melting points can be determined by techniques known in the art such as differential scanning calorimetry, a ring and ball softening test, or testing methods such as ASTM D-127 as noted in the below Examples.

Suitable waxes include, for example hydrocarbon waxes (e.g., polyethylene and polypropylene), hydrohalocarbon waxes, ester-containing waxes, synthetic waxes, and natural waxes (e.g., carnauba wax); provided, however, that the wax has a melting point in the range of about 90° C. to about 200° C. Mixtures of wax particles including mixtures of hydrocarbon wax particles and polytetrafluoroethylene (PTFE) powders can also be used. Suitable wax materials are commercially available from Micro Powders, Inc.

Preferably, the wax particles have a mean diameter in the range of about 1 to about 50 microns and more preferably in the range of about 5 to about 20 microns. The toner-receptive layer should contain no greater than 14% by weight wax based on total dry weight of the layer, since higher loadings can have a detrimental effect on surface gloss and print quality. Preferably, the toner-receptive layer comprises wax in an amount of at least 0.5 wt. % and no greater than 14 wt. % based on total dry weight of the toner-receptive layer. More preferably, the wax is present in an amount of about 1 wt. % to about 5 wt. %.

While not wishing to be bound by any theory, it is believed that the above-described toner-receptive resins and wax particles act in a synergistic manner to produce several desirable effects. Thus, the media of this invention can be used in oil-containing and oil-free electrophotographic

machines. When heated, the wax softens and part of the softened wax modifies the physical properties of the toner-receptive layer while another part of the softened wax forms a thin film between the toner-receptive layer and the fuser roll. It is thought that this softened wax compensates, at least in part, for the lack of oil in oil-free electrophotographic machines. Upon cooling, part of the wax returns to its initial role as a constituent of the toner-receptive layer, and part of it contributes to the interface between the toner-receptive layer/toner/wax layer structure and air that can cause an increase in surface glossiness of the medium. The increase in surface gloss could be due in part to a reduction in surface roughness.

The toner-receptive layer can contain anti-static agents to control static electricity build-up that may occur during the feeding, imaging, and handling of the media. The anti-static agent can modify the electrical properties of the recording medium and help provide for transferring and fusing of the toner to the medium's surface. Poorly controlled electrical properties on the imaging surface can lead to imaging defects such as image break-ups, hollow characters and deletions. Preferably, the toner-receptive layer contains anti-static agents in an amount of about 2 to about 8% by weight based on total dry weight of the toner-receptive layer. Suitable anti-static agents include sulfonated polystyrene, copolymers of dimethyl diallyl ammonium chloride, diacetone acrylamide, poly(dimethyl diallyl ammonium chloride), quaternary cellulose acetate, quaternary acrylics, inorganic salts such as ammonium chloride and sodium chloride, and other conductive materials known in the art.

In addition, the toner-receptive layer can comprise organic or inorganic particles to help control surface frictional properties of the recording medium. The particles are also useful for preventing imaging defects and reducing static electricity build-up. Useful particles include silica, calcium carbonate, kaolin, alumina, starch, olystyrene, poly(methyl methacrylate), and the like.

Coating additives, such as wetting agents, de-foaming agents, and dispersing agents, may also be incorporated in the coating formulation to improve application of the coating onto the substrate. Preferred surface wetting agents include BYK 348 and 325 (polyether modified dimethyl polysiloxane copolymers available from BYK-Chemie).

The toner-receptive layer can be prepared from either aqueous or non-aqueous-based coating formulations. The toner-receptive can be coated onto the substrate using any method known in the art including roller, rod, doctor-knife, gravure, slot-die, wire-bar, dip, and air-knife coating methods. Typically, the coat weight of the toner-receptive layer is in the range of about 1 to about 15 grams per square meter (gsm). The media of this invention can comprise single or multiple coating layers on its front surface. For example, the opaque substrate can be coated with an intermediate layer (i.e., inter-coat) and the toner-receptive coating can overlay this layer(s).

The back surface of the substrate can be non-coated, coated with the same compositions used on the front surface, or coated with a different composition than used on the front surface. If the same coating compositions are used on the front and back surfaces of the substrate, the medium may be referred to as having symmetrical coatings. If different coating compositions are used on the front and back surfaces, the medium may be referred to as having asymmetrical coatings. It can be advantageous to coat the back surface of the substrate with the same toner-receptive layer used on the front surface, thereby creating a medium that can

be imaged on either of its surfaces. A consumer can insert such products into the feed tray of a printer or copier with confidence that the "correct side is facing-up". Alternatively, other coatings can be used on the back surface of the medium to help reduce static electricity build-up during the feeding, imaging, and handling of the media and/or to improve moisture-resistance of the media.

The electrophotographic media of this invention are characterized as having good surface gloss and blocking resistance i.e. the media do not stick to each other. Particularly, the media have a surface gloss of at least 70 GU. Further, the media of this invention can be fed into color copiers and laser printers to form images having good color quality. The media are particularly suitable for use with printing devices that do not contain oil-coated fuser rolls.

The invention is further illustrated by the following examples using the below Test Methods, but these examples should not be construed as limiting the scope of the invention.

#### 20 Test Methods

##### Blocking

Non-imaged (i.e., non-printed) media samples were evaluated for blocking resistance. Each media sample was cut into four (4) pieces, each measuring 2 inches×2 inches, and the pieces were stacked on top of each other so that the coated front surface of one piece contacted the non-coated back surface of another piece. A glass plate was placed on top of the stack, and a ten (10) pound metal weight was placed on the glass plate. The stack (with weight) was placed in an oven at a temperature of about 60° C. for sixteen (16) hours. The stack was then removed from the oven, and the pieces of media were inspected to determine whether or not they stuck to each other. If there were no adhered pieces in the stack, the blocking resistance of the media was rated good. If there were some (2-4) adhered pieces in the stack, the blocking resistance of the media was rated poor.

##### 35 Surface Gloss

The surface gloss of each media sample was measured using a Micro Tri-Gloss Meter (available from BYK Gardner, Inc.) according to the standard procedures described in the instrument manual provided by the manufacturer. The surface gloss was measured on 8.5"×11" non-imaged (i.e., non-printed) sheets. The Micro-Tri Gloss Meter was calibrated at sixty (60) degrees using the standard supplied by the unit. The sample was placed on a flat surface and the surface gloss was measured at sixty (60) degrees. Measurements were made on three (3) sample sheets, and the average value was reported in terms of gloss units (GU).

As described above, the surface gloss of non-imaged sheets was measured. In addition, the sheets were printed with an image using a Xerox Docucolor 12 color copier (oil-based) or Xerox Phaser 790 laser printer (oil-free), and the surface gloss of the image on the sheet was measured using the foregoing method. The samples were printed with a test pattern image comprising colored squares. The test pattern included squares of solid primary colors (cyan, magenta, yellow, and black), and blends of primary colors (red, green, and violet).

##### Print Quality

The media samples were fed through a Xerox Docucolor 12 color copier (oil-based) or Xerox Phaser 790 laser printer (oil-free) using the bypass trays and imaged. The Xerox Docucolor 12 color copier was set at extra heavy paper mode, and the Xerox Phaser 790 laser printer was set at glossy paper mode. Printing was conducted under ambient conditions. The samples were printed with a test pattern comprising colored squares. The test pattern included squares of solid primary colors (cyan, magenta, yellow, and black), and blends of primary colors (red, green, and violet).

The printed samples were manually inspected to determine the overall quality of the printed image, and the samples were rated per the following scale:

Good—Minor variation in gloss level between printed squares, and no visible print defects.

Fair—Major variation in gloss level between printed squares and some visible print defects.

Poor—Many visible print defects such as embossing marks.

Jammed—Images could not be printed on the media because of sheet feeding problems—sheets jammed together.

## EXAMPLES

In the following Examples 1–10, a toner-receptive coating solution was prepared by mixing the following components.

|                              |             |
|------------------------------|-------------|
| Methylethyl Ketone           | 36.87 parts |
| Toluene                      | 36.87 parts |
| EPON 1007F <sup>(1)</sup>    | 24.58 parts |
| CYASTAT 609 <sup>(2)</sup>   | 1.18 parts  |
| WAX PARTICLES <sup>(3)</sup> | 0.50 parts  |

<sup>(1)</sup>EPON 1007F: an epoxy resin derived from bisphenol A and epichlorohydrin, available from Shell Chemicals Inc. EPON 1007 has a Mettler melt point (ASTM D 3461) of 120–130° C. and epoxide equivalent weight of 1700 to 2300.

<sup>(2)</sup>CYASTAT 609: a quaternary salt type cationic anti-static agent available from Cytec Industries, Inc.

<sup>(3)</sup>WAX PARTICLES: See the following Examples 1–10 for the various wax particles.

In Examples 1–10, the coating solution was applied to a surface of an 80 lb. Gloss cover paper (GARDA), available from Garda Cartiere, using a Meyer coating rod. The opacity of the paper was 89%. The coating was dried in an oven at a temperature of 250° F. for one (1) minute. The toner-receptive layer contained 96.7% epoxy resin, 1.0% wax particles, and 2.3% anti-static agent based on dry weight of the layer. The finished media samples were imaged using a Xerox Docucolor 12 color copier or Xerox Phaser 790 laser printer and evaluated as described in the above Test Methods. Results are reported below in Tables 1 and 2.

### Example 1

In this Example 1, MPP 620XF, a polyethylene wax available from Micro Powders, Inc., was used in the coating formulation. The wax has a melt point (ASTM D-127) of 114° to 116° C. and mean particle size of 5.0 to 6.0 microns.

### Example 2

In this Example 2, PROPYLTEX 325S, a polypropylene wax available from Micro Powders, Inc., was used in the coating formulation. The wax has a melt point (ASTM D-127) of 160° to 170° C. and mean particle size of 11.0 to 15.0 microns.

### Example 3

In this Example 3, MP-22XF, a straight chain hydrocarbon wax available from Micro Powders, Inc., was used in the coating formulation. The wax has a melt point (ASTM D-127) of 102° to 106° C. and mean particle size of 5.0 to 6.0 microns.

### Example 4

In this Example 4, POLYFLUO 523XF, a mixture of polyethylene wax and polytetrafluoroethylene (PTFE) powder available from Micro Powders, Inc., was used in the coating formulation. The wax has an effective melt point

(ASTM D-127) of 113° to 117° C. and mean particle size of 3.5 to 5.5 microns.

### Example 5

In this Example 5, MICROCLEAR 116, a mixture of polyethylene wax and carnauba wax available from Micro Powders, Inc., was used in the coating formulation. The wax has a melt point (ASTM D-127) of 107° to 113° C. and mean particle size of 4.5 to 5.5 microns.

### Example 6

In this Example 6, SYNFLUO 178XF, a mixture of hydrocarbon wax and polytetrafluoroethylene (PTFE) powder available from Micro Powders, Inc., was used in the coating formulation. The wax has an effective melt point (ASTM D-127) of 104° to 110° C. and mean particle size of 3.0 to 5.0 microns.

### Example 7

In this Example 7, SYNFLUO 180XF, a mixture of hydrocarbon wax and polytetrafluoroethylene (PTFE) powder available from Micro Powders, Inc., was used in the coating formulation. The wax has an effective melt point (ASTM D-127) of 104° to 110° C. and mean particle size of 3.0 to 5.0 microns.

### Example 8

In this Example 8, MPP 620F, a polyethylene wax available from Micro Powders, Inc., was used in the coating formulation. The wax has a melt point (ASTM D-127) of 114° to 116° C. and mean particle size of 9.0 to 11.0 microns.

### Example 9

In this Example 9, POLYFLUO 150, a mixture of polyethylene wax and polytetrafluoroethylene (PTFE) powder available from Micro Powders, Inc., was used in the coating formulation. The wax has an effective melt point (ASTM D-127) of 113° to 116° C. and mean particle size of 3.5 to 5.5 microns.

### Example 10

In this Example 10, MP-22, a straight chain hydrocarbon wax available from Micro Powders, Inc., was used in the coating formulation. The wax has a melt point (ASTM D-127) of 102° to 106° C. and mean particle size of 9.0 to 11.0 microns.

### Example 11

In the following Example 11, an inter-coat solution was prepared by mixing the following components.

|                           |             |
|---------------------------|-------------|
| Methylethylketone         | 60.00 parts |
| Methylpropylketone        | 15.00 parts |
| EPON 1009F <sup>(4)</sup> | 24.8 parts  |
| BYK 325                   | 0.2 parts   |

<sup>(4)</sup>EPON 1009F: an epoxy resin derived from bisphenol A and epichlorohydrin, available from Shell Chemicals Inc. EPON 1009F has a Mettler melt point (ASTM D 3461) of 130–140° C. and epoxide equivalent weight of 2300 to 3800.

In addition, a top-coat solution was prepared by mixing the following components.

|                                    |             |
|------------------------------------|-------------|
| Methylethylketone                  | 72.00 parts |
| Methylpropylketone                 | 18.00 parts |
| EPON 1007F                         | 9.10 parts  |
| CYASTAT 609                        | 0.30 parts  |
| MP 22 Wax Particles <sup>(5)</sup> | 0.80 parts  |
| BYK 325 <sup>(6)</sup>             | 0.5 parts   |

<sup>(5)</sup>MP 22: a straight chain hydrocarbon wax available from Micro Powders, Inc. The wax has a melt point (ASTM D-127) of 102° to 106° C. and mean particle size of 9.0 to 11.0 microns.

<sup>(6)</sup>BYK 325: a solution of polyether modified methylalkylpolysiloxane copolymer, available from Byk-Chemie USA, Inc.

In Example 11, the coating solutions were applied to a surface of an 80 lb. Gloss cover paper (GARDA), available from Garda Cartiere, using a Meyer coating rod. The opacity of the paper was 89%. First, the inter-coat was applied to form an intermediate layer. The coating was dried in an oven at a temperature of 250° F. for one (1) minute. The intermediate layer contained 99.56% epoxy resin and 0.44% flow agent based on dry weight of the layer. Next, the above-described top-coat solution was applied to form a toner-receptive layer. The coating layer was dried in an oven at a temperature of 250° F. for thirty (30) second. The toner-receptive layer contained 88.18% epoxy resin, 7.75% wax particles, 1.45% anti-static agent, and 2.62% flow agent based on dry weight of the layer. The finished media samples were imaged using a Xerox Docucolor 12 color copier or Xerox Phaser 790 laser printer and evaluated as described in the above Test Methods. Results are reported below in Tables 1 and 2.

#### Comparative Example A

In the following Comparative Example A, a toner-receptive coating solution was prepared by mixing the following components.

|                    |             |
|--------------------|-------------|
| Methylethylketone  | 72.00 parts |
| Methylpropylketone | 18.00 parts |
| EPON 1007F         | 9.10 parts  |
| CYASTAT 609        | 0.30 parts  |
| MP 22              | 1.60 parts  |
| BYK 325            | 0.50 parts  |

First, an inter-coat solution was applied to the surface of a paper substrate and dried as described in above Example 11. Next, the above-described top-coat solution was applied to form a toner-receptive layer. The toner-receptive layer was dried in an oven at a temperature of 250° F. for thirty (30) seconds. The toner-receptive layer contained 81.83% epoxy resin, and 14.39% wax particles based on dry weight of the layer. The finished media samples were imaged using a Xerox Docucolor 12 color copier or Xerox Phaser 790 laser printer and evaluated as described in the above Test Methods. Results are reported below in Tables 1 and 2.

#### Comparative Example B

In the following Comparative Example B, a toner-receptive coating solution was prepared by mixing the following components.

|                    |             |
|--------------------|-------------|
| Methylethylketone  | 70.00 parts |
| Methylpropylketone | 16.10 parts |
| EPON 1007F         | 9.10 parts  |
| CYASTAT 609        | 0.30 parts  |
| MP 22              | 4.00 parts  |
| BYK 325            | 0.50 parts  |

First, an inter-coat solution was applied to the surface of a paper substrate and dried as described in above Example 11. Next, the above-described top-coat solution was applied to form a toner-receptive layer. The toner-receptive layer was dried in an oven at a temperature of 250° F. for thirty (30) seconds. The toner-receptive layer contained 67.31% epoxy resin, 29.58% wax particles, 1.11% anti-static agent, and 2.00% flow agent based on dry weight of the layer. The finished media samples were imaged using a Xerox Docucolor 12 color copier or Xerox Phaser 790 laser printer and evaluated as described in the above Test Methods. Results are reported below in Tables 1 and 2.

#### Comparative Example C

In the following Comparative Example C, a toner-receptive coating solution was prepared by mixing the following components.

|                    |            |
|--------------------|------------|
| Methylethyl Ketone | 37.5 parts |
| Toluene            | 37.5 parts |
| EPON 1007F         | 25.0 parts |

The coating solution was applied to a surface of an 80 lb. Gloss cover paper (GARDA), available from Garda Cartiere, using a Meyer coating rod. The opacity of the paper was 89%. The coating was dried in an oven at a temperature of 250° F. for one (1) minute. The toner-receptive layer contained 25% epoxy resin based on dry weight of the layer. The toner-receptive layer did not contain any wax. The finished media samples were imaged using a Xerox Docucolor 12 color copier or Xerox Phaser 790 laser printer and evaluated as described in the above Test Methods. Results are reported below in Tables 1 and 2.

#### Comparative Example D

In the following Comparative Example D, a toner-receptive coating solution was prepared by mixing the following components.

|                           |            |
|---------------------------|------------|
| Methylethyl Ketone        | 37.5 parts |
| Toluene                   | 37.5 parts |
| EPON 1004F <sup>(7)</sup> | 25.0 parts |

<sup>(7)</sup>EPON 1004F: an epoxy resin derived from bisphenol A and epichlorohydrin, available from Shell Chemicals Inc. EPON 1004F has a Mettler melt point (ASTM D 3461) of 95–105° C. and epoxide equivalent weight of 800 to 950.

The coating solution was applied to a surface of a POLY-JET 112 lb. Text 6 mil clay-filled paper, available from P.H.

Glatfelter Company. The opacity of the paper was 95%. The coating was dried in an oven at a temperature of 250° F. for one (1) minute. The toner-receptive layer contained 25% epoxy resin based on dry weight of the layer. The finished media samples were imaged using a Xerox Docucolor 12 color copier or Xerox Phaser 790 laser printer and evaluated as described in the above Test Methods. Results are reported below in Tables 1 and 2.

#### Comparative Example E

Commercially available photo paper sheets from Xerox Corp. (Digital Color Photo Glossy Paper—Reorder No. 3R12155), Rochester, N.Y., were imaged using a Xerox Docucolor 12 color copier or Xerox Phaser 790 laser printer and evaluated as described in the above Test Methods. Results are reported below in Tables 1 and 2.

TABLE 1

| Sample      | (Surface Gloss)                   |                                                      |                                                    |
|-------------|-----------------------------------|------------------------------------------------------|----------------------------------------------------|
|             | Surface Gloss of Non-Imaged Media | Surface Gloss of Image on Imaged Media (Xerox DC 12) | Surface Gloss of Image on Imaged Media (Xerox 790) |
| Example 1   | 85.3                              | 81.5                                                 | 53.5                                               |
| Example 2   | 81.0                              | 80.1                                                 | 52.1                                               |
| Example 3   | 84.4                              | 77.5                                                 | 55.4                                               |
| Example 4   | 77.0                              | 91.0                                                 | 49.1                                               |
| Example 5   | 77.0                              | 87.6                                                 | 49.0                                               |
| Example 6   | 80.0                              | 85.8                                                 | 57.9                                               |
| Example 7   | 79.2                              | 85.6                                                 | 52.5                                               |
| Example 8   | 74.6                              | 90.8                                                 | 53.4                                               |
| Example 9   | 74.8                              | 91.3                                                 | 48.4                                               |
| Example 10  | 73.0                              | 90.2                                                 | 53.4                                               |
| Example 11  | 93.6                              | 83.4                                                 | 35.3                                               |
| Comp. Ex. A | 70.4                              | 74.0                                                 | 26.6                                               |
| Comp. Ex. B | 65.5                              | 79.1                                                 | 21.6                                               |
| Comp. Ex. C | 83.6                              | 90.3                                                 | 26.0                                               |
| Comp. Ex. D | 85.7                              | 83.6                                                 | No images-paper jammed                             |
| Comp. Ex. E | 97.4                              | 92.0                                                 | No images-paper jammed                             |

TABLE 2

| Sample      | (Print Quality and Blocking Resistance)     |                                           |                                         |
|-------------|---------------------------------------------|-------------------------------------------|-----------------------------------------|
|             | Print Quality of Imaged Media (Xerox DC 12) | Print Quality of Imaged Media (Xerox 790) | Blocking Resistance of Non-Imaged Media |
| Example 1   | Good                                        | Good                                      | Good                                    |
| Example 2   | Good                                        | Good                                      | Good                                    |
| Example 3   | Good                                        | Good                                      | Good                                    |
| Example 4   | Good                                        | Good                                      | Good                                    |
| Example 5   | Good                                        | Good                                      | Good                                    |
| Example 6   | Good                                        | Good                                      | Good                                    |
| Example 7   | Good                                        | Good                                      | Good                                    |
| Example 8   | Good                                        | Good                                      | Good                                    |
| Example 9   | Good                                        | Good                                      | Good                                    |
| Example 10  | Good                                        | Good                                      | Good                                    |
| Example 11  | Good                                        | Good                                      | Good                                    |
| Comp. Ex. A | Fair                                        | Fair                                      | Good                                    |
| Comp. Ex. B | Fair                                        | Fair                                      | Good                                    |
| Comp. Ex. C | Good                                        | Poor                                      | Good                                    |
| Comp. Ex. D | Fair                                        | No images-paper jammed                    | Poor                                    |
| Comp. Ex. E | Good                                        | No images-paper jammed                    | Poor                                    |

As shown in above Table 1, for non-imaged media and media printed with an image using the Xerox DC-12 color

copier (oil-based), surface gloss tends to be relatively high (greater than 70 GU). In contrast, when a non-oil based machine such as the Xerox 790 laser printer is used, the surface gloss of the printed image tends to be relatively low (less than 60 GU). However, even when such a non-oil-based machine is used, the media of this invention are capable of providing images having relatively good surface gloss (at least 35 GU) versus other media. In addition, as shown in above Table 2, the non-imaged media of this invention exhibit good blocking resistance in contrast to other media. Further, when the media of this invention are printed with images using the Xerox DC-12 color copier or Xerox 790 laser printer, the print quality of the image is good in contrast to images produced on other media.

#### 15 What is claimed is:

1. An electrophotographic recording medium comprising an opaque substrate having a surface coated with a toner-receptive layer comprising a resin selected from the group consisting of epoxy and polyester resins having a melting point in the range of about 105° C. to about 200° C., and wax having a melting point in the range of about 90° C. to about 200° C., wherein the amount of said wax in the layer is no greater than 14% by weight based on total weight of the layer, said recording medium having a surface gloss of at least 70 GU.
2. The recording medium of claim 1, wherein the opaque substrate is a cellulosic material.
3. The recording medium of claim 1, wherein the opaque substrate is a polymeric film.
4. The recording medium of claim 1, wherein the toner-receptive layer comprises an epoxy resin.
5. The recording medium of claim 3, wherein the epoxy resin, is derived from bisphenol A and epichlorohydrin.
6. The recording medium of claim 1, wherein the toner-receptive layer comprises a polyester resin.
7. The recording medium of claim 1, wherein the melting point of the resin is in the range of about 110° C. to about 170° C.
8. The recording medium of claim 1, wherein the wax is selected from the group consisting of hydrocarbon, hydrohalocarbon, ester-containing, synthetic, and natural waxes.
9. The recording medium of claim 8, wherein the wax is a hydrocarbon wax selected from the group consisting of polyethylene and polypropylene waxes.
10. The recording medium of claim 9, wherein the wax is a natural wax.
11. The recording medium of claim 1, wherein the wax has a melting point in the range of about 90° C. to about 150° C.
12. The recording medium of claim 1, wherein the toner-receptive layer further comprises an anti-static agent selected from the group consisting of cationically conductive polymers and anionically conductive polymers.
13. The recording medium of claim 1, wherein the toner-receptive layer further comprises pigment particles selected from the group consisting of silica, calcium carbonate, kaolin, aluminum hydroxide, starch, polystyrene, and poly(methyl methacrylate) particles.
14. The recording medium of claim 1, wherein the substrate has a thickness in the range of about 2 to about 8 mils.
15. The recording medium of claim 1, wherein the coat weight of the toner-receptive layer is the range of about 1 to about 15 grams per square meter.
16. The recording medium of claim 1, wherein the amount of wax in the layer is in the range of about 1% to about 5% by weight based on the weight of the layer.

**13**

17. The recording medium of claim 1, wherein the wax comprises wax particles having a mean diameter size in the range of about 1 to about 50 microns.

18. A process for producing an image on an electrophotographic recording medium comprising the steps of:

- 5 a) providing an electrophotographic recording medium comprising an opaque substrate having a surface coated with a toner-receptive layer comprising a resin selected from the group consisting of epoxy and polyester resins having a melting point in the range of about 105° C. to about 200° C., and wax having a melting point in the range of about 90° C. to about 200° C., wherein the amount of said wax in the layer is no greater than 14%

**14**

by weight based on total weight of the layer, said recording medium having a surface gloss of at least 70 GU;

- b) applying toner to form an image on the surface of the medium; and
- c) treating the medium with heat to fuse the toner to the medium.

10 19. The process of claim 18, wherein the medium is passed between heated rollers to fuse the toner to the medium.

20. The process of claim 19, wherein the heated rollers are non oil-coated.

\* \* \* \* \*